



US008877605B1

(12) **United States Patent**  
**Xie et al.**

(10) **Patent No.:** **US 8,877,605 B1**  
(45) **Date of Patent:** **Nov. 4, 2014**

(54) **SILICON SUBSTRATE FABRICATION**

(71) Applicants: **Yonglin Xie**, Pittsford, NY (US);  
**Carolyn R. Ellinger**, Rochester, NY (US); **Mark D. Evans**, Rochester, NY (US); **Joseph Jech, Jr.**, Webster, NY (US)

(72) Inventors: **Yonglin Xie**, Pittsford, NY (US);  
**Carolyn R. Ellinger**, Rochester, NY (US); **Mark D. Evans**, Rochester, NY (US); **Joseph Jech, Jr.**, Webster, NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **13/860,557**

(22) Filed: **Apr. 11, 2013**

(51) **Int. Cl.**

**H01L 21/76** (2006.01)  
**B41J 2/16** (2006.01)

(52) **U.S. Cl.**

CPC ..... **B41J 2/1626** (2013.01)  
USPC ..... **438/424**; 438/427; 438/443; 438/444;  
257/E21.004; 257/E21.345

(58) **Field of Classification Search**

None

See application file for complete search history.

(56) **References Cited**

U.S. PATENT DOCUMENTS

|              |      |         |                              |
|--------------|------|---------|------------------------------|
| 7,208,800    | B2   | 4/2007  | Chung et al.                 |
| 8,519,478    | B2 * | 8/2013  | Rassel et al. .... 257/335   |
| 8,541,820    | B2 * | 9/2013  | Hayasaki et al. .... 257/225 |
| 2009/0096835 | A1   | 4/2009  | Nagata                       |
| 2009/0147049 | A1   | 6/2009  | Lee et al.                   |
| 2009/0273647 | A1   | 11/2009 | Kwon et al.                  |

FOREIGN PATENT DOCUMENTS

CN 102344114 2/2012

\* cited by examiner

Primary Examiner — Zandra Smith

Assistant Examiner — Khanh Duong

(74) Attorney, Agent, or Firm — William R. Zimmerli

(57) **ABSTRACT**

A method of etching a silicon substrate includes providing a silicon substrate including a first surface and a second surface. A plurality of grooves spaced apart from each other are etched from the first surface of the silicon substrate. A dielectric material is deposited on the first surface of the silicon substrate and into the plurality of grooves. A hole through the silicon substrate is etched from the second surface of the substrate to the dielectric material. A portion of the hole is located between the plurality of grooves.

**4 Claims, 13 Drawing Sheets**



**FIG. 1**





FIG. 2g



FIG. 2h



FIG. 2c



FIG. 2d



FIG. 3f



FIG. 3g



FIG. 3a



FIG. 3b



FIG. 3h



FIG. 3i



FIG. 3c



FIG. 3d

**FIG. 3e****FIG. 3j**

**FIG. 4****FIG. 5**



FIG. 6c



FIG. 6d



FIG. 6a



FIG. 6b



FIG. 7b



FIG. 7a

***FIG. 8a******FIG. 8b***

**FIG. 9a**

(PRIOR ART)

**FIG. 9b**

(PRIOR ART)



**FIG. 10a**



**FIG. 10b**

**FIG. 10C****FIG. 10D**

## 1

## SILICON SUBSTRATE FABRICATION

## CROSS REFERENCE TO RELATED APPLICATIONS

Reference is made to commonly-assigned, U.S. patent application Ser. No. 13/860,560, entitled "SILICON SUBSTRATE MEMS DEVICE", filed concurrently herewith.

## FIELD OF THE INVENTION

This invention relates generally to micro-fluid ejection assemblies and, in particular, to ejection devices having flow features formed therein using Micro-Electrical-Mechanical Systems (MEMS) processing techniques.

## BACKGROUND OF THE INVENTION

Micro-fluidic ejection devices typically include a silicon substrate material that includes "flow features," for example, fluid openings, fluid passages, holes, trenches, or depressions, formed therein. These flow features may be formed by a wide variety of micromachining techniques including sand blasting, wet chemical etching and reactive ion etching. As these devices become smaller, such as for ink jet printhead applications, micromachining of the substrates becomes a more critical operation.

One micromachining technique of particular interest is a silicon dry etch technique known as Deep Reactive Ion Etch (DRIE). DRIE has the potential to create deep and narrow holes through a silicon wafer. DRIE can routinely produce aspect ratios as high as 25:1, which can be critical in creating holes that are closely spaced, such as is needed for high-resolution ink jet printhead devices. DRIE goes by many names in the literature; however, herein we are referring specifically to the Bosch process that features sequential ionic plasma etch and passivation layer deposition. This technique offers high drilling rates with vertical sidewalls and high aspect ratio (height/width).

Some of the drawbacks of the DRIE process include an aspect ratio dependent etching rate. This means that the rate of drilling is slower for small diameter holes than it is for larger diameter holes. Variability in etching rate is also found when comparing holes made in the center of the silicon wafer to the edges of the wafer (commonly referred to as the bulls-eye effect). Microloading is another known issue in which isolated holes will drill somewhat faster than holes that are situated nearby to other holes. When holes are being drilled all the way through the silicon wafer from one surface to the other, these rate differences may not matter too much. However, certain MEMS applications require that a silicon substrate have holes that are drilled down to an insulating layer, which serves as an etch stop or as a device functional layer. When hole drilling stops at an insulating layer on the surface of the wafer, such as is found in Silicon on Insulator (SOI) substrates, variability in the etch rate often leads to additional defects.

In particular, when SOI wafers are etched using DRIE, notching occurs. Referring to FIG. 9a, notching, which is present in region 930, is the phenomenon of localized undercutting of the silicon at the silicon/insulator boundary. It is widely believed that this phenomenon is caused by local charging of the insulating layer 960 by plasma ions in region 980 which causes lateral deflection of the ionic species resulting in lateral etching of the sidewalls in region 930. Notching can also be understood, more elementarily, as caused by over etching, especially where some of the holes in a wafer reach

## 2

the insulating layer before the etching process is complete due to etching rate variability described previously.

A number of countermeasures to reduce or even prevent notching have been proposed. One widely used technique is to observe when the hole approaches the insulating layer and then alter the DRIE parameters to reduce the etching rate. This approach works well when there are uniform hole etching rates, but even then, requires difficult or complex monitoring techniques to know when to reduce the etch rate without unduly sacrificing productivity.

Several approaches using changes in pulse duty cycle or frequency have been found to reduce notching, but changes in optimized etching process parameters are likely to have a negative impact on etching characteristics such as etch rate or anisotropy. Another approach is to add a metallization layer to the insulator to avoid charge build up, but that adds manufacturing complexity, especially if that metal layer must be removed after the DRIE is complete.

As such, there is an ongoing need to develop a solution in which the insulating layer itself reduces or even prevents notching preferably without adding additional complexity or cost to the process or the finished product.

## SUMMARY OF THE INVENTION

According to an aspect of the invention, a method of etching a silicon substrate includes etching a plurality of grooves spaced apart from each other on a first surface of a silicon substrate. A dielectric material is deposited on the first surface of the silicon substrate and into the plurality of grooves. A hole is etched through the silicon substrate from the second surface of the substrate to the dielectric material. A portion of the hole is located between the plurality of grooves. The dielectric material in the grooves acts to stop the lateral etching that contributes to notching, thereby reducing, limiting, or even preventing a notching defect in the silicon substrate.

According to another aspect of the invention, the starting location and size of the hole on the second surface of the silicon wafer are determined by providing a mask on the second surface of the silicon substrate prior to etching the hole through the silicon substrate from the second surface of the substrate to the dielectric material. The mask defines the hole diameter which is smaller than the spacing between the grooves. The mask is aligned relative to the plurality of grooves so that etching through the silicon substrate from the second surface of the substrate creates a through hole that is aligned with respect to the plurality of grooves.

According to another aspect of the invention, at least a portion of the dielectric material located between the plurality of grooves can be removed either prior to or after completion of the hole formation. In one example embodiment of the invention, the plurality of grooves, formed to contain the dielectric material by acting to stop lateral etching, can be distinct portions of a continuous groove. The continuous groove can have various shapes including, for example, a rectangle with rounded corners, an oval, or a circular shape when viewed from a direction perpendicular to the first surface of the silicon substrate.

## BRIEF DESCRIPTION OF THE DRAWINGS

In the detailed description of the example embodiments of the invention presented below, reference is made to the accompanying drawings, in which:

FIG. 1 is a flow chart describing process steps for etching a silicon substrate according to an example embodiment of the invention;

FIGS. 2a through 2d and 2e through 2h are cross-sectional views, taken along line A-A', and plan views, respectively, of one example embodiment of the invention showing formation of a silicon structure with a through hole;

FIGS. 3a through 3e and 3f through 3j are cross-sectional views, taken along line A-A', and plan views, respectively, of another example embodiment of the invention showing formation of a silicon structure with a through hole;

FIG. 4 is a cross sectional view of an example embodiment of a MEMS device of the invention;

FIG. 5 is a cross sectional view of another example embodiment of a MEMS device of the invention;

FIGS. 6a through 6d are plan views of example embodiments of the plurality of grooves of the invention;

FIGS. 7a and 7b are plan views of another example embodiment of a MEMS device of the invention;

FIGS. 8a and 8b are a cross-sectional view, taken along line A-A', and a plan view, respectively, of another example embodiment of a MEMS device of the invention;

FIGS. 9a and 9b are cross-sectional views of prior art devices; and

FIGS. 10a through 10d are cross-sectional views of example embodiments of MEMS devices of the invention.

#### DETAILED DESCRIPTION OF THE INVENTION

Deep dry etching of silicon is now a routine process in MEMS fabrication. Deep Reactive Ion Etching uses sequential etch and deposition steps. The etching step uses an isotropic plasma etch, typically using sulfur hexafluoride, SF<sub>6</sub>, for silicon. Sulfur hexafluoride gas is injected into a low-pressure chamber, containing the silicon wafer to be processed, and then energized with a spark discharge to create a plasma, which contains ions. The wafer is typically coated with a photoresist mask, which is resistant to ion etching, to define the regions where the hole is to be drilled. Gaps in the mask determine the location and size of the etched hole.

As the etching proceeds, a cycle of etching and passivation is used to achieve the high aspect ratio desired to drill small holes through a relatively thick silicon wafer. Typical chemically inert passivation materials include fluorocarbons, similar to Teflon™. The coating of the hole by the passivation layer discourages the sidewalls of the hole from further etching through the protected layer. However, the directional bombardment ions erodes the passivation layer at the bottom of the hole resulting in further etching of the silicon in the vertical direction. These etch/deposit steps are repeated many times over resulting in a large number of very small isotropic etch steps taking place only at the bottom of the etched pits. The end result is a deep, narrow hole or trench.

Charge build up in the bottom of the holes or the sidewall of the holes is prevented by the inherent conductivity of silicon which allows charge deposited (or induced) by the ionic species to bleed away or be neutralized by counter charge in the wafer walls. As a result, the ionic bombardment of the plasma SF<sub>6</sub> proceeds as expected throughout the growth of the hole. In the presence of an insulating layer, which, for example, might be present on the backside of the wafer, the deposited charge can accumulate. The resulting change in the electric field in the hole can then drive the reactive ions into the side walls resulting in lateral erosion or notching (also referred to as footing). FIGS. 9a and 9b, described in more detail below, show examples of lateral erosion or notching.

In the case of a single hole being drilled in a silicon wafer, adjustment to the etch rate as it approaches the insulating layer can reduce or ultimately prevent notching if the etch

process is promptly stopped when the hole is complete. As described earlier, however, in the more typical case where many holes are being fashioned at the same time in a wafer; and especially if there is variation in the hole sizes, density and radial location on the wafer, some holes will be complete and starting to notch while other holes are still not complete. This means that simply adjusting the etch process can not completely prevent notching.

In addition to being an insulating layer, the dielectric layer present in Silicon on Insulator (SOI) devices or as membranes in MEMS devices is typically resistant to dry etching. Thus, it has been determined that in the present invention, the dielectric layer can act as a stop for the vertical etching. Referring to FIG. 1, a flow chart is shown describing the steps of one example embodiment of the invention for etching a silicon substrate, in which the dielectric layer also helps to reduce or even prevent notching.

The process begins with providing the silicon substrate, step 1. Then, a plurality of shallow grooves is produced on the first surface of the silicon substrate, typically using, for example, a photoresist mask and a wet etch process, step 10. Then, a dielectric material is deposited onto the first surface of the substrate, step 20. The dielectric layer can be deposited using any standard process. For example, spin coating can be used when materials such as spin-on-glass (SOG) are being deposited. The dielectric material also can be deposited using other systems and techniques. For example, vapor deposition systems and techniques including chemical vapor deposition (CVD) and atomic layer deposition (ALD) can be used. The dielectric material also can be deposited using sputtering or reactive sputtering techniques. The dielectric material can be organic or preferably inorganic. Useful inorganic dielectric materials include SiO<sub>2</sub>, TiO<sub>2</sub>, SiC, Si<sub>3</sub>N<sub>4</sub>, ZrO, TaO, and others known in the art. Because of the presence of the grooves, the dielectric material also fills the plurality of grooves, step 20. The dielectric material can completely fill the grooves, as shown in FIGS. 2 and 3, or only coat the walls of the grooves, leaving a portion of the groove unfilled. The location of the grooves on the first surface of the substrate must be aligned with the location of the holes in the dry etch mask on the second surface of the substrate. It is immaterial in which order the masks on the first and second surface of the substrate are created. Standard techniques exist, that are well known in the art, to align first and second surface masks (commonly referred to as front and backside masks). With the second surface of the substrate mask in place and the first surface of the substrate grooves coated with dielectric, the holes can now be etched through from the second surface of the substrate to the first surface of the substrate using DRIE, step 30.

FIGS. 2a-2d and 2e-2h are cross-sectional views, taken along line A-A', and plan views, respectively, of one example embodiment of the invention showing formation of a silicon structure including a hole through the silicon wafer 200. FIGS. 2a-2c and 2e-2g show the formation of dielectric coated grooves on the first surface of the substrate. FIGS. 2a and 2e show silicon wafer 200 before processing. This corresponds to step 1 of FIG. 1. The first surface of the substrate 200 is labeled 210 and the second surface of the substrate is labeled 220.

FIGS. 2b and 2f show the wafer after the etching process is complete to produce the plurality of grooves 250 in the first surface 210 of the silicon substrate. This corresponds to step 10 of FIG. 1. FIGS. 2c and 2g show the first surface 210 now coated with the dielectric layer 260. As shown in FIGS. 2c and 2g, dielectric layer 260 readily flows into grooves 250. This is

a necessary characteristic of the dielectric material to enable the present invention. This corresponds to step 20 of FIG. 1.

FIGS. 2d and 2h show the finished wafer after the hole 280 is drilled using DRIE from the second surface 220 of the substrate 200 to the first surface 210 of the substrate 200. The DRIE stops where it contacts the dielectric layer 260. This corresponds to step 30 of FIG. 1. Details of the prevention of notching by the dielectric in the grooves will be discussed later. As shown in FIG. 2d, the entirety of hole 280 is contained within the boundary defined by the inner surface 251 of the groove 250. This is an essential feature of the first embodiment of the invention.

FIGS. 3a-3e and 3f-3j are cross-sectional views, taken along line A-A', and plan views, respectively, of another example embodiment of the invention showing formation of a silicon structure with a through hole through the silicon 300 and the dielectric layer 360. FIGS. 3a, 3b, 3c, 3f, 3g, and 3h are identical to FIGS. 2a, 2b, 2c, 2e, 2f, and 2g.

FIGS. 3d and 3i show the formation of a small hole 370 in the dielectric layer 360. Hole 370 is formed by a conventional process, for example, mask formation, wet etching, and mask removal. After creation of the through hole 370, the DRIE process then forms hole 380 starting from the second surface 320 of the silicon substrate 300. Alternatively, hole 380 can be formed first, followed by the formation of hole 370. The resulting structure, shown in FIGS. 3e and 3j, has many applications. For example, the structure shown in FIGS. 3e and 3j can be used in fluidic devices including, for instance, ink jet printheads. FIG. 3j shows the concentric and size relationship of the membrane through hole 370, the silicon through hole 380 and the groove 350 for this example embodiment.

Referring to FIG. 4, another example embodiment of a MEMS device of the present invention is shown. This embodiment is similar to the structure shown in FIG. 2d which included a suspended dielectric membrane 460 over a deep hole 480 in the silicon substrate. In the embodiment shown in FIG. 4, however, the grooves 450 are coated with a different notch stop material 455 than used for the membrane. This is advantageous in cases where there are other material deposition and patterning steps prior to the deposition and patterning of the membrane material. The notch stop material can be a dielectric material and serves the same function as the dielectric coated grooves discussed above. The pattern for the additional notch stop material can be identical to that of the grooves, as shown in FIG. 4, or may be different as long as the notch stop material 455 coats the walls of the groove 450.

Referring to FIG. 5, another example embodiment of a MEMS device of the present invention is shown. This embodiment is similar to the structure shown in FIG. 3e. In the embodiment shown in FIG. 5, however, a suspended dielectric membrane 560 includes through hole 570 in the membrane that is over (as shown in the figure) and aligned with a through hole 580 in the silicon substrate. In the embodiment shown in FIG. 5, the grooves 550 are coated with a different notch stop material 555 than used for the membrane. As discussed with reference to FIG. 4, this is advantageous in cases where there are other material deposition and patterning steps prior to the deposition and patterning of the membrane material.

The present invention contemplates various patterns for the plurality of grooves on the first surface of the silicon substrate that can be effective for reducing or even preventing notching. Referring to FIGS. 6a-6d, plan views of example embodiments of the plurality of grooves of the present invention are shown. In FIGS. 6a, 6c and 6d, example embodiments are shown in which the plurality of grooves is distinct portions of

a continuous groove. FIG. 6a shows a circular groove 650 in the first side 610 of the silicon wafer 600. Circular grooves have the advantage of reducing the size of the groove for a given radius of the groove pattern. Referring back to FIG. 2h, the entirety of the hole 280 must be inside the inner wall of the groove 251. A concentric groove circle and deep hole will accomplish this provided that the expected tolerance stack up errors on alignment of the front side and back side masks are within acceptable limits. FIG. 6c shows an oval shape for the groove. This is particularly useful when there is a known tolerance issue that is greater in one direction (for example, the vertical direction as shown in FIG. 6c) when compared to the orthogonal direction (the horizontal direction as shown in FIG. 6c). FIG. 6d shows a rectangular shape with curved corners for the groove pattern that increases the tolerance for alignment errors at the expense of slightly longer groove paths which can result in a greater quantity of dielectric material being used to coat or fill the grooves. The rectangular shape is also suitable for applications where the deep drilled hole itself has a rectangular shape, as shown, for example, in FIG. 7b.

In some MEMS applications, it is desirable to create features with deep trenches rather than holes. This is easily done using DRIE by simply changing the mask pattern for the deep hole on the second surface of the silicon substrate. When it is desired to create or drill deep trenches, groove patterns, for example, one of the patterns shown in FIG. 6b, are appropriate for trenches when compared to holes. It should be understood that there are variations and modifications of groove patterns that are within the scope of the present invention.

In many MEMS applications, holes or trenches are not created in isolation. For example, many fluidic devices, including most ink jet printheads, include an array of closely spaced holes. In this case, as well as other similar designs, a series of interconnected grooves 750 can be provided, or created, for the first surface 710 of the silicon substrates 700 shown in FIGS. 7a and 7b. The interconnected plurality of grooves 750 on the first surface 710 of silicon substrate 700 are shown in FIG. 7a. FIG. 7b shows the series of deep etch holes 780, 782, 784. As shown in FIGS. 7a and 7b, the grooves and the holes include a rectangular aspect although other shapes can be used depending on the application contemplated.

Referring now to FIG. 8, an example embodiment that addresses a significant practical issue in using dielectric filled grooves to reduce or even prevent notching is shown. In applications, the tolerance stack up error for aligning the grooves on the first surface of the silicon substrate to the hole produced using DRIE and a mask on the second surface of the silicon substrate can be large enough to be potentially problematic. Referring back to FIG. 2d, if the deep hole 280 is sufficiently off center when compared to the groove 250, there is a risk that a portion of the hole will reach the first side of the wafer beyond the inner boundary 251 of the groove 250. If this were to happen, substantial notching can occur. If, on the other hand, the groove diameter is made much larger so as to preclude the possibility of the hole location 280 exceeding the boundary 251 of groove 250, the dielectric can be too far from the edge of the hole to reduce or prevent substantial notching. In other words, the distance from the outer edge of the hole 280 to the inner edge, the boundary 251, of the groove 250 can be greater than the extent of notching that occurs.

FIGS. 8a and 8b are a cross-sectional view, taken along line A-A', and a plan view, respectively, of a portion of another example embodiment of a MEMS device of the present invention that provides an additional countermeasure to this tolerance issue. As shown, an inner groove 840 helps to insure that

the location of the notch preventing dielectric will be sufficiently close to the outer surface of the deep hole. In the event that the deep hole in some locations is located outside of the groove **840**, the hole will still be contained inside the outer groove **850** so as to reduce or prevent notching from occurring regardless of the tradeoff between tolerance stack-up and size of the groove.

The following discussion provides an explanation for the mechanism of how the dielectric filled grooves reduce or even prevent notching. This explanation, however, should not be considered as in any way restricting the scope of the present invention. FIGS. **9a** and **9b** are cross-sectional views of prior art examples that include notching. FIG. **9a** shows a single hole **980** in a SOI device in which over-etching has caused severe notching in region **930** under (as shown in the figure) the dielectric material **960**. FIG. **9b** shows an example of a failure effect that can result from notching. In FIG. **9b**, there are two closely spaced holes **980a** and **980b** that are not supposed to be in fluidic communication. The portion **901** of the silicon wafer **900** separating the holes **980a**, **980b** is supposed to prevent fluidic communication. As shown, however, the center post **901** has been sufficiently eroded in region **940** due to severe notching **930** in region **940** to allow fluid to pass from one passage **980a** to the other passage **980b**.

Referring to FIGS. **10a-10d**, cross-sectional views of example embodiments of MEMS devices of the present invention are shown which overcome the issues associated with the prior art devices. Although the insulating nature of the dielectric layer contributes to the lateral deflection of the plasma ionic species in DRIE, the dielectric material itself is highly resistant to etching. As shown in FIG. **10a**, when the lateral erosion that results in notching reaches the inner side wall of the dielectric filled groove, it is stopped from proceeding any further by the resistance of the dielectric to the etching. In this sense, notching of the silicon is not actually prevented, but the extent of the notching is limited or reduced. FIG. **10b** shows how effective this can be to effectively prevent the kind of failure effect shown in FIG. **9b**. In FIG. **10b**, the grooves in the inner post **101** of the silicon wafer **100** effectively prevent the notching from proceeding across the entire top of the center post **101**. Thus, region **145** of silicon wafer **100** is protected and fluidic separation between the holes **180a** and **180b** is maintained.

FIG. **10c** illustrates the result when the tolerance issues are considered. As shown, hole **180** is somewhat off-center compared to the groove pattern **150**. As a result, notching still occurs in region **134** but is controlled in region **132**. While this can be undesirable in some applications, it typically does not result in a failure mode, since the notching is reduced or contained within acceptable limits. FIG. **10d** illustrates a more severe tolerance issue in which notching in region **136** is about to escape the confines of the groove **150**. In this situation, a second groove pattern, outside of the first groove pattern (as shown in FIGS. **8a** and **8b**) helps to contain the notch.

The invention has been described in detail with particular reference to certain preferred embodiments thereof, but it will be understood that variations and modifications can be effected within the scope of the invention.

## PARTS LIST

1 step  
10 step  
20 step  
30 step  
100 silicon substrate

110 first surface  
120 second surface  
130 notch stopped on groove  
132 notch stopped on groove  
5 134 notch offset from groove  
136 notch under groove  
145 silicon wall  
150 groove  
160 dielectric material  
10 180 through hole  
200 silicon substrate  
210 first surface  
220 second surface  
250 groove  
15 251 inner surface of the groove  
260 dielectric material  
280 through hole  
300 silicon substrate  
310 first surface  
20 320 second surface  
350 groove  
360 dielectric material  
370 hole  
380 through hole  
400 silicon substrate  
410 first surface  
420 second surface  
450 groove  
30 455 notch stop material  
460 dielectric material  
480 through hole  
500 silicon substrate  
510 first surface  
35 520 second surface  
550 groove  
555 notch stop material  
560 dielectric material  
570 hole  
40 580 through hole  
600 silicon substrate  
610 first surface  
620 second surface  
650 circular groove  
45 650 oval groove  
670,675 parallel elongated groove  
672,674 parallel elongated groove  
650 rounded rectangular groove  
700 silicon substrate  
50 710 first surface  
720 second surface  
750 continuous groove for multiple through holes  
780 first through hole  
782 first through hole  
55 784 first through hole  
800 silicon substrate  
810 first surface  
820 second surface  
840 first groove  
60 850 second groove  
900 silicon substrate  
910 first surface  
920 second surface  
930 notch  
65 940 missing silicon wall (merged notches)  
960 dielectric material  
980 through hole

The invention claimed is:

1. A method of etching a silicon substrate comprising:
  - providing a silicon substrate including a first surface and a second surface;
  - etching a plurality of grooves spaced apart from each other 5 from the first surface of the silicon substrate, adjacent grooves of the plurality of grooves having a spacing when viewed from a direction perpendicular to the first surface of the silicon substrate;
  - depositing a dielectric material on the first surface of the 10 silicon substrate and into the plurality of grooves;
  - providing a mask on the second surface of the silicon substrate that defines a dimension of interest that is smaller than the spacing between the adjacent grooves when viewed from the direction perpendicular to the first 15 surface of the silicon substrate, and aligning the mask relative to the plurality of grooves so that the dimension of interest is between adjacent grooves; and
  - etching a hole defined by the dimension of interest through the silicon substrate from the second surface of the substrate to the dielectric material, the hole being contained 20 within the confines of the adjacent grooves.
2. The method of claim 1, further comprising:
  - removing at least a portion of the dielectric material located 25 between the plurality of grooves.
3. The method of claim 1, wherein the plurality of grooves are distinct portions of a continuous groove.
4. The method of claim 3, wherein the continuous groove has one of a rectangle with rounded corners, an oval, and a circular shape when viewed from a direction perpendicular to 30 the first surface of the silicon substrate.

\* \* \* \* \*